

## 1

3,746,585

## TITANIUM-BASE ALLOYS

Richard Ernest Goosey, Aldridge, England, assignor to  
 Imperial Metal Industries, London, England  
 No Drawing. Continuation of abandoned application Ser.  
 No. 836,625, June 25, 1969. This application Dec. 7,  
 1971, Ser. No. 205,728  
 Int. Cl. C22f 1/18; C22c 15/00  
 U.S. Cl. 148—32.5

4 Claims

## ABSTRACT OF THE DISCLOSURE

Alloys of the titanium plus 1.5–3.5% copper type, suitable for strip and sheet manufacture, are given increased strength, without detriment to their other properties, by the addition of up to 5% in total from the group of 0.25–5% of aluminium, zirconium and tin and 0.1–1 silicon. The alloys are age-hardenable.

This is a continuation of application Ser. No. 836,625, filed June 25, 1969, now abandoned.

## BACKGROUND OF THE INVENTION

This invention relates to titanium-base alloys and in particular to alloys suitable for the manufacture of sheet and strip.

A titanium alloy suitable for sheet having moderate strength has been known for some years, and this alloy is a binary alloy containing nominally 2.5% copper. The ductility of the alloy is satisfactory for forming operations and welding can be carried out without adversely affecting ductility. The alloy is age hardenable to an ultimate tensile strength of about 50 tonf./sq. in. under certain conditions but such a level of strength is not adequate for certain applications and no alternative sheet alloy with a suitable combination of properties exists.

We have found that the composition of the above-mentioned alloy can be so modified that a higher strength can be obtained without detriment to other properties, in particular, formability.

## SUMMARY OF THE INVENTION

According to the present invention a titanium-base alloy consists of 1.5–3.5% by weight copper and up to 5% in total of one or more of the following elements 0.25–5.0% aluminium, 0.25–5.0% zirconium, 0.25–5.0% tin, 0.1–1.0% silicon, balance titanium, apart from impurities.

## DESCRIPTION OF THE PREFERRED EMBODIMENT

Ternary alloys within the above ranges have been prepared containing elements in the following amounts:

Titanium-2.5% copper+0.5, 1.0, 1.5, 2.0 and 3.0% aluminium  
 Titanium-2.5% copper+1.0, 3.0 and 5.0% zirconium  
 Titanium-2.5% copper+1.0, 3.0 and 5.0% tin  
 Titanium-2.5% copper+0.25 and 0.5% silicon

Quaternary alloys containing the following have been prepared:

Titanium-2.5% copper+0.5, 1.0 and 1.5% aluminium +1.0% zirconium  
 Titanium-2.5% copper+0.5, 1.0 and 1.5% aluminium +0.25% silicon

Other alloys prepared include:

Titanium-2.5% copper-1.0% zirconium-0.25% silicon +0.5, 1.0 and 1.5% aluminium.

## 2

All these alloys possessed improved strength compared with the previously known alloy without significantly affecting the ductility and weldability.

The best range of compositions has been found experimentally to be within the following limits in respect of aluminium, zirconium and silicon.

|            | Percent  |
|------------|----------|
| Aluminium  | 1.5–3.0  |
| Zirconium  | 1.0–3.0  |
| 10 Silicon | 0.25–0.5 |

and these are the preferred ranges.

The addition of the elements mentioned herein to the basic titanium-2.5% copper alloy has been found to suppress the increase in hardness during aging if the amounts specified are exceeded. The addition of up to 5% tin completely suppresses age hardening in titanium-2.5% copper. Within the limits specified, improvement in tensile properties can be obtained and in the preferred compositions, the maximum increase is obtained.

Titanium alloys normally contain carbon, oxygen and nitrogen as impurities and in the alloys in accordance with the invention, carbon and nitrogen are maintained at normal impurity levels but oxygen may be present up to 0.25% with advantage, since the tensile strength is thereby increased by 3 to 4 tonf./in.<sup>2</sup> without significantly affecting ductility. Oxygen is normally present in the range 0.13–0.18%.

The preferred alloys having a good combination of properties are those having the following compositions:

30 Titanium-2.5% copper-1.5% aluminium  
 Titanium-2.5% copper-2.0% aluminium  
 Titanium-2.5% copper-1.0% aluminium-1.0% zirconium-0.25 silicon.

35 Alloys in accordance with the invention are age hardenable after solution treatment at a temperature of 775° C. or more depending upon the composition. The preferred alloys are solution treated at 810–820° C. and the aging temperature is in the range 425–450° C.

40 In heat-treatment tests on the preferred alloys, maximum hardening was obtained by aging at 425° C. The highest aging response was observed on titanium-2.5% copper-1.5% aluminium, which increased in strength from 44.5 tonf./in.<sup>2</sup> to about 57 tonf./in.<sup>2</sup>, an increase of 12.5 tonf./in.<sup>2</sup>. On the other hand, the titanium-2.5% copper-2.0% aluminium alloy, which had a solution treated strength 4.5 tonf./in.<sup>2</sup> higher than the 1.5% aluminium alloy, only increased in strength by 8.5 tonf./in.<sup>2</sup> from 49.1 tonf./in.<sup>2</sup> to 57.6 tonf./in.<sup>2</sup>. The quaternary alloy had a solution treated strength of 47.1 tonf./in.<sup>2</sup> and exhibited an aging response of some 11 tonf./in.<sup>2</sup>. Although a fall in reduction of area values was evident after aging, all three alloys possessed high ductility at the maximum strength level.

55 Age-hardening characteristics of the three alloys at 425° C. were quite different. Tensile strength of the titanium-2.5% copper-1.5% aluminium alloy tended to increase progressively with aging time and was accompanied by the steady growth of a coherent precipitate which was about 600 Å. in length after 192 hours at 425° C.

60 The titanium-2.5% copper-2.0% aluminium alloy did not increase in strength to any extent during the first 72 hours at 425° C. and then appeared to increase quite significantly in the next 48 hours. The number of nuclei formed in this alloy appeared to be smaller than on titanium-2.5% copper-1.5% aluminium, but their rate of growth seemed to be more rapid, precipitates being around 800 Å. in length after 192 hours at 425° C.

65 In contrast to the ternary titanium-copper-aluminium alloys, titanium-2.5% copper-1.0% aluminium-1.0% zir-

conium-0.25% silicon hardened rapidly during the first 48 hours at 425° C., but did not increase in tensile strength to any great extent thereafter. The substantial hardening during the early stages of aging was associated with extensive nuclei formation which grew only slowly on further aging, a precipitate size of 200 Å being recorded after 192 hours at 425° C.

Raising the aging temperature by 10° C. to 435° C. had a pronounced effect on nucleation and growth of the precipitate in all three alloys and consequently on aging response. Non-coherent overaged precipitates of 1500 Å and 2500 Å length were noted in the 1.5% and 2.0% aluminium alloys after 96 hours at this temperature. On the other hand precipitates in the zirconium-silicon bearing alloys were coherent and 650 Å in size.

After 96 hours at 450° C., precipitates in all three alloys were non-coherent and larger than those formed after a similar time at 435° C.

The intended use of alloys in accordance with the invention is as sheet, and it is desirable that sheet should have adequate bending properties and good weldability in addition to good tensile strength. The preferred alloys possess such as combination of properties.

A summary of properties after solution treating at 820°

of the preferred alloys are consistent with this value having regard to their higher tensile strength.

The properties of solution treated and welded, and of welded and aged sheet, tested with the weld transverse to the test piece axis were quite satisfactory, and revealed no evidence of embrittlement in the weld area.

The preferred alloys have considerably greater tensile strength than the titanium-2.5% copper alloy and increases in strength of up to 10 tonf./in.<sup>2</sup> have been observed. With oxygen contents of up to 0.25%, sheet alloys having a tensile strength of 60 tonf./in.<sup>2</sup> and over are obtainable.

Adequate ductility is maintained in these alloys and with the highest tensile strengths elongation values of about 17-18% can be expected. The alloys are cold formable.

When heat-treated, alloys according to the invention exceed 55 tonf./in.<sup>2</sup>, which is 10% greater than the nominal 50 tonf./in.<sup>2</sup> of the binary alloy and dependent upon composition, may reach 20% greater tensile strength.

Elevated temperature tensile tests show that the alloys of the invention have appreciably higher strength at 300° C. and 400° C. after heat-treatment compared with the binary alloy.

TABLE I

| Alloy                               | Solution treated properties        |                               |                                    |                | Properties after aging at 425° C.  |                               |                                    |                |                                             |             |
|-------------------------------------|------------------------------------|-------------------------------|------------------------------------|----------------|------------------------------------|-------------------------------|------------------------------------|----------------|---------------------------------------------|-------------|
|                                     | 0.1% PS,<br>tonf./in. <sup>2</sup> | TS,<br>tonf./in. <sup>2</sup> | Percent<br>elong.<br>4 $\sqrt{So}$ | RA,<br>percent | 0.1% PS,<br>tonf./in. <sup>2</sup> | TS,<br>tonf./in. <sup>2</sup> | Percent<br>elong.<br>4 $\sqrt{So}$ | RA,<br>percent | Aging<br>period<br>(hrs.)                   | Test piece  |
| Ti-2.5, Cu-1.5, Al                  | 32.7                               | 44.5                          | 26                                 | 31             | 46.9                               | 57.6                          | 20                                 | 27             | 192                                         | Rolled rod. |
| Ti-2.5, Cu-2.0, Al                  | 35.7                               | 49.1                          | 21                                 | 34             | 47.4                               | 57.0                          | 20                                 | 32             | 144                                         | Do.         |
| Ti-2.5, Cu-1.0, Al-1.0, Zr-0.25, Si | 35.3                               | 47.1                          | 19                                 | 40             | 44.3                               | 58.3                          | 23                                 | 31             | 192                                         | Do.         |
| Ti-2.5, Cu                          | 31.2                               | 42.5                          | 29                                 | 47             | 40.0                               | 51.5                          | 24                                 | 40             | 24 hrs. at 400° C. and<br>8 hrs. at 475° C. |             |

TABLE II

| Nominal composition, weight percent | Heat-treatment procedure                              | Test material                       | 0.1% PS,<br>tonf./in. <sup>2</sup> | 0.2% PS,<br>tonf./in. <sup>2</sup> | TS,<br>tonf./in. <sup>2</sup> | Percent<br>elong.<br>on $\frac{1}{2}$ in. | Limiting<br>bend<br>radius t |
|-------------------------------------|-------------------------------------------------------|-------------------------------------|------------------------------------|------------------------------------|-------------------------------|-------------------------------------------|------------------------------|
| Ti-2.5, Cu-1.5, Al                  | Solution treated $\frac{1}{2}$ hr. at 820° C. A.C.    | Parent sheet                        | 29.3                               | 31.4                               | 39.6                          | 20                                        | 3.0                          |
|                                     | Solution treated and aged 168 hrs. at 425° C.         | do                                  |                                    |                                    | 52.7                          | 20                                        |                              |
|                                     | Solution treated and welded.                          | Weld transverse to test piece axis. | 34.8                               | 35.9                               | 41.4                          | 12                                        | 3.0                          |
|                                     | do                                                    | Weld parallel to test piece axis.   |                                    |                                    | 42.5                          | 25                                        |                              |
|                                     | Solution treated, welded, aged 168 hrs. at 425° C.    | Weld transverse to test piece axis. |                                    |                                    | 50.9                          | 16                                        |                              |
| Ti-2.5, Cu-2, Al                    | Solution treated $\frac{1}{2}$ hr. at 820° C. A.C.    | Parent sheet                        | 37.1                               | 37.2                               | 44.0                          | 20                                        | 2.35                         |
|                                     | Solution treated and welded.                          | Weld transverse to test piece axis. | 36.0                               | 36.8                               | 42.9                          | 10                                        | 2.6                          |
|                                     | do                                                    | Weld parallel to test piece axis.   |                                    |                                    | 45.2                          | 28                                        |                              |
|                                     | Solution treated, welded and aged 168 hrs. at 425° C. | Weld transverse to test piece axis. |                                    |                                    | 52.1                          | (b)                                       |                              |
| Ti-2.5, Cu-1, Al-1, Zr-0.25, Si     | Solution treated $\frac{1}{2}$ hr. at 805° C. A.C.    | Parent sheet                        | 37.1                               | 37.4                               | 44.4                          | 26                                        | 2.5                          |
|                                     | Solution treated and aged 168 hrs. at 425° C.         | do                                  |                                    |                                    | 55.1                          | 18                                        |                              |
|                                     | Solution treated and welded.                          | Weld transverse to test piece axis. | 35.3                               | 26.7                               | 44.4                          | 10                                        | 3.2                          |
|                                     | do                                                    | Weld parallel to test piece axis.   |                                    |                                    | 46.7                          | 26                                        |                              |
|                                     | Solution treated, welded and aged 168 hrs. at 425° C. | Weld transverse to test piece axis. |                                    |                                    | 55.8                          | 14                                        |                              |

\* Parent sheet failure at end of gauge length. <sup>b</sup> Fractured outside gauge length.

NOTE.—All tests transverse to final sheet rolling direction except those with weld parallel to gauge length.

C. in the case of ternary alloys or 810° C. in other cases and after age hardening is given in Table I. Tests were made on rolled rod to facilitate test piece manufacture. Tests made on sheet, including welded sheet, are shown in Table II. The limiting bend test indicates the minimum radius, expressed as a multiple of the thickness of the sheet, around which the test piece could be bent cold without cracking.

By way of comparison it should be mentioned that titanium-2.5% copper, when heat-treated to a tensile strength of about 50 tonf./in.<sup>2</sup> can be bent around a radius of 3 times its thickness. The bending properties

I claim:

1. A solution-treated age-hardened titanium base alloy in sheet form having a tensile strength exceeding 55 tonf./square inch and a limiting bend radius of not more than 3T and good weldability, said alloy consisting essentially of, by weight, 1.5-3.5% copper, 1.5-3.0% aluminum, 1.0-3.0% zirconium, 0.25-0.5% silicon, balance titanium, apart from impurities, the total amount of aluminum, zirconium and silicon not exceeding 5%.

2. A titanium-base alloy as in claim 1 containing 0.13-0.25% oxygen.

3. A titanium-base alloy as in claim 1 containing 2.5% copper, 1.0% aluminum, 1.0% zirconium, 0.25% silicon, balance titanium apart from impurities.

4. A titanium-base alloy as in claim 1 solution treated at 810-820° C. and aged at 425-450° C.

References Cited

UNITED STATES PATENTS

|           |        |               |          |    |
|-----------|--------|---------------|----------|----|
| 2,868,640 | 1/1959 | Butler        | 75-175.5 |    |
| 2,867,534 | 1/1959 | Jaffee et al. | 75-175.5 | 10 |
| 2,777,768 | 1/1957 | Busch et al.  | 75-175.5 |    |

FOREIGN PATENTS

|           |         |               |          |    |
|-----------|---------|---------------|----------|----|
| 653,682   | 12/1962 | Canada        | 75-175.5 |    |
| 1,057,578 | 2/1967  | Great Britain | 75-175.5 | 15 |

|           |        |               |          |
|-----------|--------|---------------|----------|
| 771,952   | 4/1957 | Great Britain | 75-175.5 |
| 1,108,039 | 3/1968 | Great Britain | 75-175.5 |
| 594,813   | 3/1960 | Canada        | 75-175.5 |

OTHER REFERENCES

WADC Technical Report 58-328, "Development of Active-Euctactoid Base Alloys," October 1958, pp. 1-7, 10, 11, 32 and 33.

CHARLES N. LOVELL, Primary Examiner

U.S. Cl. X.R.

75-175.5; 148-133

UNITED STATES PATENT OFFICE  
CERTIFICATE OF CORRECTION

Patent No. 3,746,585 Dated July 17, 1973

Inventor(s) RICHARD ERNEST GOOSEY

It is certified that error appears in the above-identified patent and that said Letters Patent are hereby corrected as shown below:

In the heading, after "This application Dec. 7, 1971,  
Ser. No. 205,728" insert --Claims priority, Application  
Great Britain, July 1, 1968, 31369/68--.

Signed and sealed this 14th day of May 1974.

(SEAL)  
Attest:

EDWARD M.FLETCHER, JR.  
Attesting Officer

C. MARSHALL DANN  
Commissioner of Patents